

May 23, 1961

2,985,569

L. W. GENDVIL  
ELECTROLYTIC METHOD AND MEANS FOR  
PRODUCTION OF REFRACTORY METAL  
Filed July 30, 1956



Fig. 1.



Fig. 2.

INVENTOR  
Leonard W. Gendvil

BY

*H. H. Hammons*

AGENT

## 1

2,985,569

## ELECTROLYTIC METHOD AND MEANS FOR PRODUCTION OF REFRAC-

Leonard W. Gendvil, Dongan Hills, Staten Island, N.Y., assignor to National Lead Company, New York, N.Y., a corporation of New Jersey

Filed July 30, 1956, Ser. No. 600,758

5 Claims. (Cl. 204—64)

This invention relates to the electrolytic production of refractory metals. More particularly, it relates to the production of high purity zirconium metal by an electrolytic process adapted specifically to the production of zirconium metal on a commercial scale.

There are many compounds of refractory metals which are found in nature but which are extremely difficult to reduce to the metallic state. In many instances it is relatively easy to convert such compounds to the halides of the refractory metals by halogenation processes, but it is difficult to produce the refractory metals from their respective halides. Included in the group of metals which fall within the class known as refractory metals are titanium, zirconium, vanadium, niobium, tantalum, molybdenum, tungsten, thorium and uranium.

Some of these refractory metals have heretofore been produced from their compounds by thermal reduction methods employing pressure and a reducing metal, while others have been produced by direct chemical reduction of the halide employing metallic sodium or metallic magnesium as reducing agents. While these methods have produced such metals, they suffer from a fundamental economic disadvantage in that the cost of the reducing metal employed, such as sodium or magnesium, is relatively high and the processes are expensive and cumbersome to operate.

The production of titanium metal by a direct electrolytic process has now been accomplished, but despite the fact that titanium and zirconium metals are each in group IVa of the periodic table attempts to produce zirconium by such process have not been successful. The instant application relates to an improved direct electrolytic process by which zirconium metal may be produced and is characterized by the discovery of novel operational features, whereby zirconium metal of high purity may be produced on a commercial scale.

An object, therefore, of the present invention is to provide a superior electrolytic process for producing zirconium metal of high purity from zirconium metal halides.

A further object is to provide an improved method for operating an electrolytic cell whereby coarse crystalline non-pyrophoric zirconium metal may be produced economically in relatively large quantities and in a commercially feasible manner.

A still further object of the invention is to provide a superior electrolytic cell for producing highly ductile non-pyrophoric zirconium metal on a commercial scale.

These and other objects of this invention will become apparent from the following more complete description thereof and the accompanying drawings in which:

Fig. 1 is a vertical cross section of an electrolytic cell embodying a cathode in the form of a conical metal member; and

Fig. 2 is a plan view of the cell on section line 2—2 of Fig. 1.

In its broadest aspects, the instant invention contemplates a semi-continuous method for producing a refrac-

## 2

tory metal, and in particular zirconium metal, in an electrolytic cell having a cathode, an anode and a fused salt bath by feeding vaporous  $ZrCl_4$  into said bath below the surface thereof an in immediate proximity to a cathodic surface while simultaneously passing direct current between the anode and said cathodic surface at a rate synchronized with the  $ZrCl_4$  addition so that the amount of current is sufficient to reduce the  $ZrCl_4$  being added to zirconium metal; and depositing the zirconium metal as an adherent mass of coarse crystalline metal on the cathodic surface while maintaining the bath substantially free of reduced zirconium values except in the immediate vicinity of the cathodic surface.

More particularly, the invention contemplates the deposition of a coarse crystalline deposit of non-pyrophoric zirconium metal on the interior surfaces of a bell-shaped cathode having a perforated bottom by introducing the vaporous  $ZrCl_4$  into the interior of the bell-shaped cathode below the surface of the electrolyte, and maintaining 10 the adherent mass of zirconium metal and the perforated cathode perforative and the bath exteriorly of the bell-shaped cathode substantially free of reduced zirconium values.

As has been disclosed in the electrolytic art relating to 25 the production of titanium, the halides of titanium and in particular the tetravalent chlorides and bromides of titanium, while not readily soluble in a fused salt bath, nevertheless can be electrolytically reduced to titanium metal by passing direct current through the cell at a rate 30 synchronized with the rate of titanium metal halide addition to the fused salt bath so that the amount of current is sufficient to reduce a substantial portion, if not all of the titanium metal halide, substantially directly to titanium metal. This technique is hereinafter referred to as substantially direct electrolysis of titanium metal halides in 35 a fused salt bath.

According to the present invention, it has been discovered that zirconium metal may also be produced by 40 direct electrolysis of zirconium halides and that recoveries of a coarse crystalline non-pyrophoric metal on a commercially practical scale are obtained by confining the zirconium metal halide in a fused salt bath to the immediate vicinity of a cathodic surface such that the zirconium metal will be deposited substantially in toto thereon; and 45 that the production of this superior form of Zr metal is effected by controlling the operating conditions of a particular cell and the type and orientation of the cathodic surface relative to the anode and the point of introduction of the zirconium halide into the fused salt bath such that the zirconium metal deposit is maintained perforative throughout a given run.

The phrase "confined to the immediate vicinity of the cathode," as used herein, will be understood to mean that the zirconium halide introduced into the fused salt bath 55 is not permitted to diffuse throughout the molten salt electrolyte but is directed toward and maintained substantially in intimate contact with a cathodic surface whereby the zirconium halide values are reduced to metal in the form of a zirconium metal deposit on the cathodic surface. The preferred method and means by which the zirconium halide may be confined to the immediate vicinity of a cathodic surface and the metal deposit formed thereon forms the subject matter of the instant invention and is described hereinafter in detail.

The phrase "operating conditions," as used herein, has 60 reference to the control which must be maintained over variables such as time, temperature of the fused salt bath, the cathode current density, current-to- $ZrCl_4$  feed ratio, cathode design, and zirconium content of the electrolyte within the cathode in order to carry out the step 65 of maintaining the deposit of zirconium metal in perforative form.

In this connection it should be explained that by perforative means a porous crystalline type of deposit as distinguished from a dense solid deposit. While there is some doubt as to the exact nature of the electrolytic chemistry involved, it has been found that direct electrolytic reduction of zirconium halide values to zirconium metal as large deposits of ductile non-pyrophoric crystalline metal can be accomplished on a commercial scale by the use of a cathodic surface, preferably in the form of a metal cone, having a grill or screen across its open base, into which the  $ZrCl_4$  is introduced below the surface of the electrolyte. It may be postulated that ionic currents proceed from the anode through the screen in the bottom of the cathodic cone and through the voids in the perforative deposit of zirconium metal to the inside of the cone where zirconium ions may be found and reduced to zirconium metal on the inner walls of the cone. Contrary to what one might expect, a major portion of the ionic current does not stop at the exterior surfaces of the cathodic cone but apparently continues on through the cathodic screen base of the cone and through the relatively infinite number of substantially parallel paths in the perforative deposit of zirconium metal to the interior of the cone.

In order to describe more clearly the details of the instant invention, the process will be specifically illustrated by describing the production of zirconium metal from zirconium tetrahalide.

Referring to Fig. 1, the apparatus shown consists of a cell container 10 heated by graphite electrodes 11-11. The cell container is filled or partially filled with an electrolyte 12 in which is suspended a pair of graphite anodes 13-13 between which is supported a cathode-member indicated generally at 15. The fused salt electrolyte, sometimes referred to hereinafter as a fused salt bath, comprises preferably a molten halide salt of an alkali or alkaline earth metal, including magnesium, particularly the chlorides of said metals which may be employed singly or in combinations. Mixtures of these halides which form low melting point eutectics are most convenient to employ such as, for example, mixtures of sodium chloride and strontium chloride, sodium chloride and lithium chloride, sodium chloride and barium chloride, sodium chloride and magnesium chloride or mixtures thereof. In general, the temperature of the fused salt bath may vary within the range of from 600° C. to 950° C. depending upon the particular salts used, the type of metal being deposited and the construction of the cell itself. For the production of zirconium metal using a sodium chloride bath, operating temperatures within the range of from 750°-850° C. have been found preferable.

Referring again to the cathode member 15, the latter comprises a feed pipe 16 which is used for introducing the tetrachloride into the electrolyte and which extends coaxially of a metal pipe 17 connected at its upper end to the negative side of a current source; and having a bell-type enlargement at its lower end comprising preferably a metal cone 18 provided with a screen or grid 19 across its open base. The cone may be formed of iron or nickel, and inasmuch as it is integral with or connected electrically to the cathodic metal pipe 17, it itself is cathodic. An important control in the operation of the cell is that of introducing the incoming zirconium chlorides into the fused salt bath at a point in the cathodic cone 18 below its apex, and to this end the feed pipe 16 extends down into the cone far enough so that the lower extremity of the pipe terminates close to the screen base of the cone. As a consequence, the zirconium chlorides are brought into intimate contact with the cathodic surfaces which confine and restrict the dispersion of the zirconium chlorides to that portion of the electrolyte within the interior of the cone such that zirconium metal is deposited on the bottom and walls thereof in the form of relatively large particles of ductile metal.

It is significant that whereas substantially cylindrical perforated metal baskets (iron or titanium metal) have been used successfully to produce coarse crystalline deposits of titanium metal, it has been found that for the production of Zr metal the use of a bell-type member having a screen over its open bottom end is a definite aid in the deposition of crystalline non-pyrophoric zirconium metal.

The screen or grid base 18 of the cathodic cone is also iron or nickel and is a relatively coarse screen, the apertures of which may vary from 8 to 256 per sq. inch area of the screen, a preferred screen size being 100 apertures to the square inch. In this connection the overall area of the screen 18 is the area used in computing the cathode current density which may vary from 200 to 800 amperes per square foot.

For reduction to take place on the inside or inner surfaces of the zirconium deposit, it is necessary that the ionic current pass through the perforative deposit of zirconium metal to the interior of the cone where the zirconium ions are found. As the deposit increases in thickness, it offers increased resistance to the passage of the ionic current which for constant rate of reduction requires higher voltage and amperage. This in turn results in lower current efficiencies. In brief, the nature of the operation is such that it will cut itself off. However, if operated under proper conditions a deposit of practical thickness and porosity will be formed on the inner walls of the cone.

In carrying out the process of the instant invention, the metal halide is added, preferably in vapor form, to the fused salt bath concurrently with the addition of current. In order that the halide may be added at a substantially constant rate, it is preferred to meter the halide in the vapor state.

As mentioned above, in order to reduce zirconium tetrachloride to metal, a predetermined amount of current must be passed concurrently through said cell at a rate synchronized with the rate of zirconium tetrachloride addition. A theoretically sufficient current will comprise about four faradays of electricity passed concurrently through the cell while approximately one mol of zirconium tetrachloride is being introduced into the cell. In actual practice, however, it has been found desirable to add a quantity of electricity somewhat in excess of the theoretical amount in order to make up the current loss caused by said reactions in the cell and to account for variations in the rate of feed of the zirconium tetrachloride. While in theory it would be sufficient to add about 4-5 faradays of electricity to maintain efficient cell operation, in practice variations in sublimation rate, and hence the feed rate of vaporous zirconium tetrachloride may necessitate modification of the theoretical current-to-feed ratio such that five to fifteen faradays of electricity are required per mole of zirconium tetrachloride.

An alternative expediency is to vary the current to fit the  $ZrCl_4$  feed rate and to use the cell E.M.F. as an indication of the current-to-feed ratio that prevails in the system at any given instant. For a cathode having a desirably perforative deposit a cell E.M.F. of 2.3-2.6 volts will be indicative of a current-to-feed ratio of about 5.6 faradays/mole while an E.M.F. of 2.7-2.8 is indicative of a current-to-feed ratio of 8-12 faradays per mole. Moreover, it is known that the cell E.M.F. is a function of the concentration of reduced chlorides in the melt, and that a low E.M.F., i.e. 2.3-2.6 volts, is indicative of high concentrations of reduced chlorides in the melt while a high E.M.F., i.e. 2.7-2.8 volts, is indicative of low concentrations of reduced chlorides in the melt. The higher concentrations corresponding to low E.M.F. tend to produce a massive deposit of zirconium whereas the lower concentrations of reduced zirconium chlorides produce a dendritic deposit.

In order to illustrate the invention further the following examples are given.

*Example I*

Using a cell similar to that shown in Figure 1 a conical nickel cathode having a nickel screen over its open base with  $\frac{1}{16}$ " apertures spaced  $\frac{1}{10}$ " on centers and having a nickel feed pipe for the introduction of zirconium tetrachloride vapors into the interior of the cathodic cone adjacent the bottom thereof was lowered into a fused salt electrolyte consisting of 400 pounds of sodium chloride maintained at a temperature of about 900° C. Zirconium tetrachloride vapors were then introduced at the rate of 170 grams per hour into the feed pipe of the cathodic nickel cone. Concurrently, an electric current equivalent to 6.1 faradays per mole of zirconium tetrachloride was passed through the cell. This amount of current was in effect sufficient to completely reduce the zirconium tetrachloride to zirconium metal. In order to obtain substantially 6.1 faradays per mole of zirconium tetrachloride introduced, 125 amperes with an impressed voltage of approximately 6 volts was required. The cathode current density was about 400 amperes per square foot. The run was made for a period of 6 hours during which time the deposit of zirconium metal remained perforative and the apertures in the screen open. At the end of this period the introduction of zirconium tetrachloride vapor was stopped and no further current was passed through the electrolyte. The cathodic cone was withdrawn from the cell and zirconium metal was found deposited on the walls of the cathode in the form of an irregular perforative tenacious mass composed of relatively large crystals. The zirconium metal was removed from the cell and cooled in a chamber having an inert atmosphere. The cooled deposit was leached and the dried leached zirconium metal was recovered as coarse crystals weighing 344 grams having a definite metallic luster and being quite ductile. A sample prepared by arc melting these crystals possessed a Brinell hardness of 198. About 87% of the zirconium values introduced as zirconium tetrachloride were recovered as zirconium metal. The cell E.M.F. was 2.4 volts.

*Example II*

Using a cell similar to that shown in Fig. 1, a conical nickel cathode provided with a nickel screen over its base having  $\frac{1}{16}$ " apertures spaced  $\frac{1}{10}$ " on centers and having a nickel feed pipe for introducing zirconium tetrachloride vapors into the cathode was lowered into a fused salt electrolyte consisting of 400 lbs. of sodium chloride maintained at a temperature of about 900° C. Zirconium tetrachloride vapors were introduced into the interior of the cathode below the surface of the electrolyte at the rate of 95 grams per hour and zirconium metal was deposited on the walls of the basket as relatively large coarse particles of metal. Concurrently an electric current equivalent to 9.3 faradays per mole of zirconium tetrachloride was passed through the cell. This amount of current was in effect sufficient to completely reduce the zirconium tetrachloride to zirconium metal. In order to obtain substantially 9.3 faradays per mole of zirconium tetrachloride introduced, 100 amperes with an impressed voltage of approximately 5.6 volts was required. The cathode current density was about 400 amperes per square foot. The run was made for a period of 6 hours during which time the deposit of zirconium metal remained perforative and the apertures in the screen open. The cathode was withdrawn from the cell and zirconium metal was found deposited on the interior walls of the cone in the form of an irregular perforative tenacious mass composed of relatively large crystals. The leached zirconium metal recovered, as described in the preceding example, weighed 148 grams which analyzed substantially 99.8% zirconium and possessed a Brinell hardness of about 222. The cell E.M.F. was 2.8 volts.

*Example III*

Using the same technique described in Examples I and II with a salt bath comprising 400 pounds of 30 mole per-

cent KCl, 34 mole percent  $\text{SrCl}_2$  and 36 mole percent NaCl, and a cathodic iron cone having a nickel screen with  $\frac{1}{32}$ " perforations spaced 256 holes to the square inch and a  $\frac{3}{4}$ " feed pipe,  $\text{ZrCl}_4$  was fed into the electrolyte

- 5 at the rate of 120 grams per hour, the temperature of the bath being 700° C. Electric current equivalent to 7.2 faradays per mole of  $\text{ZrCl}_4$  was passed through the cell, the amount of current required being 100 amperes at an impressed voltage of about 6 volts. The cathode current density was about 400 amperes per square foot and the run was continued uninterruptedly for 7.3 hours. The coarse zirconium metal produced by this run weighed approximately 200 grams, the Brinell hardness of which was about 342.
- 10 15 It has been clearly shown by the description of the instant invention and by the examples presented that refractory metals may be obtained by passing a refractory metal halide into an electrolytic cell by means of a conical nickel cathode at a rate synchronized with the electric current addition such that the amount of electricity added per mole of refractory metal halide measured in faradays is numerically substantially greater than the number of halide atoms present in the said refractory metal halide molecule; and that by confining the reduced halides to the immediate vicinity of the cathode while concurrently retaining the zirconium metal deposit on the cathodic surfaces, high recoveries of ductile relatively coarse zirconium metal may be obtained. Thus, the electrolytic process of the instant invention employs simple and inexpensive apparatus whereby it is possible to produce refractory metals economically and continuously.

20 25 30 35 While this invention has been described and illustrated by the examples shown, it is not intended to be strictly limited thereto, and other modifications and variations may be employed within the scope of the following claims.

I claim:

1. A method for producing zirconium metal in an electrolytic cell having an anode, bell-type cathode having 40 a perforated bottom, and a fused salt bath consisting essentially of salt selected from the group consisting of alkali metal halides, alkaline earth metal halides, magnesium halides and mixtures thereof comprising the steps of: introducing  $\text{ZrCl}_4$  below the surface of said bath into the interior of said bell-type cathode, passing electric current between the anode and said bell-type cathode at a rate synchronized with the  $\text{ZrCl}_4$  addition so that the amount of current is sufficient to reduce the  $\text{ZrCl}_4$  being added to metal and depositing an adherent mass of zirconium metal in the interior of the bell-type cathode, while maintaining the electrolyte exteriorly of the cathode substantially free of reduced zirconium values.
2. A method for producing zirconium metal in an electrolytic cell having an anode and a fused salt bath 55 consisting essentially of salt selected from the group consisting of alkali metal halides, alkaline earth metal halides, magnesium halides and mixtures thereof comprising the steps of: submerging a bell-type cathode having a perforated bottom in said fused bath, introducing  $\text{ZrCl}_4$  below the surface of said bath into the interior of said bell-type cathode, passing electric current between the anode and cathode at a rate synchronized with the  $\text{ZrCl}_4$  addition so that the amount of current is sufficient to reduce the  $\text{ZrCl}_4$  being added to metal, depositing zirconium metal in the interior of the cathode, meanwhile maintaining the bottom of said cathode and the deposit of zirconium metal in perforative form and maintaining the electrolyte exteriorly of the cathode substantially free of reduced zirconium values.
3. A method for producing zirconium metal in an electrolytic cell having an anode and a fused salt bath consisting essentially of salt selected from the group consisting of alkali metal halides, alkaline earth metal halides, magnesium halides and mixtures thereof comprising the 60 65 70 75 steps of: submerging a bell-type cathode having a per-

forated bottom in said fused bath, introducing  $ZrCl_4$  below the surface of said bath into the interior of said cathode, passing electric current between the anode and cathode at a rate synchronized with the  $ZrCl_4$  addition so that the amount of current is sufficient to reduce the  $ZrCl_4$  being added to metal, depositing an adherent mass of zirconium metal in the interior of the cathode, and simultaneously controlling the operating conditions of said cell such that said adherent mass of zirconium metal is perforative and the electrolyte exteriorly of the cathode is substantially free of reduced zirconium values.

4. A method for producing zirconium metal in an electrolytic cell having an anode and a fused salt bath consisting essentially of salt selected from the group consisting of alkali metal halides, alkaline earth metal halides, magnesium halides and mixtures thereof comprising the steps of: submerging a cone-shaped cathode having a perforated bottom in said fused bath, introducing  $ZrCl_4$  below the surface of said bath into the interior of said cathodic cone, passing electric current between the anode and cathodic cone at a rate synchronized with the  $ZrCl_4$  addition so that the amount of current is sufficient to reduce the  $ZrCl_4$  being added to metal, depositing an adherent mass of zirconium metal in the interior of the cathodic cone, and maintaining the current-to-feed ratio within the range of from 5-15 faradays per mole and the cathode current density within the range of from 200-800 amperes per square foot such that said adherent mass of zirconium is perforative and the electrolyte exteriorly of the cathodic cone is substantially free of reduced zirconium values.

5. A method for producing zirconium metal in an electrolytic cell having an anode and a fused salt bath consisting essentially of salt selected from the group consisting of alkali metal halides, alkaline earth metal halides, magnesium halides and mixtures thereof comprising the steps of: submerging a cone-shaped cathode having a screen over its open bottom end in said fused bath, introducing  $ZrCl_4$  into the interior of said cathodic cone adjacent the screen at the bottom thereof, passing electric current between the anode and cathodic cone at a rate synchronized with the  $ZrCl_4$  addition such that the cell E.M.F. is in the range of from 2.7-2.8 volts and the cathode current density is within the range of from 400-500 amperes per square foot, depositing an adherent mass of zirconium metal in the interior of the cathodic cone, and maintaining said adherent mass of zirconium metal in perforative form and the electrolyte exteriorly of the cathodic cone substantially free of reduced zirconium values.

## References Cited in the file of this patent

## UNITED STATES PATENTS

|    |           |                  |       |               |
|----|-----------|------------------|-------|---------------|
| 25 | 513,661   | Vautin           | ----- | Jan. 30, 1894 |
|    | 631,253   | Gooch            | ----- | Aug. 15, 1899 |
|    | 1,050,902 | Acker            | ----- | Jan. 21, 1913 |
|    | 2,749,295 | Svanstrom et al. | ----- | June 5, 1956  |
| 30 | 2,760,930 | Alpert et al.    | ----- | Aug. 28, 1956 |
|    | 2,801,964 | Opie et al.      | ----- | Aug. 6, 1957  |